

# United States Patent Office.

THOMAS L. REED, OF PROVIDENCE, RHODE ISLAND, ASSIGNOR TO THE ATLANTIC TUBING COMPANY, OF THE SAME PLACE.

*Letters Patent No. 71,787, dated December 3, 1867; antedated November 21, 1867.*

## IMPROVED COMPOSITION FOR PRESERVING ANIMAL INTESTINES.

The Schedule referred to in these Letters Patent and making part of the same.

TO ALL WHOM IT MAY CONCERN:

Be it known that I, THOMAS L. REED, of the city and county of Providence, and State of Rhode Island, have invented a new and improved Composition for Preserving Animal Intestines and membranous tissues in a natural, moist condition; and I do hereby declare that the following is a full, clear, and exact description of the same.

In a previous patent, granted to David K. Hoxsie and myself, September 27, 1864, and numbered 44,425, a method is described of preserving or curing animal intestines, and utilizing the same in the manufacture of flexible gas-tubing, to render the same impervious to illuminating-gas, or, in other words, gas-tight. Also, in another patent, granted subsequently, to said Hoxsie and myself, to wit, on the 21st day of November, A. D. 1865, and numbered 51,052, a description is recited of a means for preserving the intestine, so cured and utilized, in its naturally moist condition by means of a compound of glycerine and glue, in suitable proportion, properly prepared and applied.

The invention in this instance relates to the same subject, and is calculated to subserve the same purpose as that last mentioned, that is to say, to prevent the membrane from becoming dry and husky, and in consequence liable to crack and permit the gas to escape, as it would be likely to do from the bending and other usage to which this article is subjected; and my present invention consists of other compounds, with a base of glycerine, which possess the non-drying properties of glycerine and glue in a more eminent degree, and which, besides, are cheaper, and on some accounts are better adapted to the purpose intended.

These compounds, and that of glycerine and glue as well, contribute nothing of an impervious character to the intestine or to the article of tubing wherein the intestine is used for that purpose. On the contrary, the imperviousness is wholly conceded to the membrane as a natural property of its own, which is perfect as compared with any simply artificial means, and which it is the office only of the said compound to maintain in all its natural perfection in this new sphere of usefulness.

The material from which this moistening effect is mainly derived is glycerine, but owing to its subtle nature, it cannot be retained next to the intestine unless it is combined with some material which will give it consistency the more like paste or jelly, and less like oil; and it was simply for the purpose of imparting to the glycerine the requisite consistency that the article of glue has heretofore combined therewith, as above alluded to. But it is found in practice that other substances than glue are better adapted to preserve intact the desirable moistening properties of the glycerine, while at the same time they are equally instrumental in reducing the same to the proper consistency, besides being familiar and cheaper commodities, and these are substantially as follows:

First, glycerine and molasses, equal parts of each, mingled while cold, and afterwards heated to the boiling-point, then allowed to cool, when it is fit for use.

Second, glycerine and flour; the flour made into a paste by boiling ( $\frac{1}{4}$ ) one-quarter by weight of water with the quantity of flour, and mix while warm with the glycerine, equal parts of each.

Third, glycerine and gum-tragacanth; the gum dissolved in water in the usual way to make a paste; afterwards sift the paste and mix, cold, with an equal quantity of glycerine.

Fourth, glycerine and gum-arabic; gum-arabic dissolved in water to the consistency of molasses, and afterwards mingled with the glycerine, equal parts of each.

Fifth, a compound, the "four" ingredients as follows: gum-tragacanth, one pound; gum-arabic, one pound; flour, two pounds; glycerine, eight pounds. Mingle together and heat to the boiling-point, 212°.

Sixth, glycerine and gum-substitute; add to the gum water enough to moisten it, and boil steadily from one (1) to three (3) days—the longer time the better—then add an equal quantity by weight of glycerine.

Besides the above, I have successfully employed a compound of Irish moss and molasses, mixed with glycerine, the moss being first soaked in water, as in its use for culinary purposes, and after it is dissolved mingle therewith an equal part by weight of molasses, and with the two an equal quantity by weight of glycerine. Heat the whole to the boiling-point, and when cool it is ready for use.

What I claim, and desire to secure by Letters Patent, is—

The use of glycerine and the several commodities herein enumerated in compound, substantially as and for the purpose specified.

In witness whereof, I have hereunto set my hand, this twentieth day of November, A. D. 1866.

THOMAS L. REED,

Witnesses:

ISAAC A. BROWNELL,  
D. K. HOXSIE.